

June 4, 1968

T. L. JOHNSTON ET AL

3,386,862

HIGH STRENGTH STRUCTURAL STEEL

Filed June 22, 1966

2 Sheets-Sheet 1



FIG. 1



FIG. 2

RAYMOND C. BOETTNER  
RICHARD H. BUSH  
THOMAS L. JOHNSTON  
ARTHUR J. McEVILY, JR.  
INVENTORS

BY *John R. Faulkner*  
*Thomas H. Oster*

ATTORNEYS

June 4, 1968

T. L. JOHNSTON ET AL

3,386,862

HIGH STRENGTH STRUCTURAL STEEL

Filed June 22, 1966

2 Sheets-Sheet 1



FIG. 3

RAYMOND C. BOETTNER  
RICHARD H. BUSH  
THOMAS L. JOHNSTON  
ARTHUR J. McEVILY, JR.

INVENTORS

BY *John R. Faulkner*  
*Thomas H. Oster*

ATTORNEYS

3,386,862

## HIGH STRENGTH STRUCTURAL STEEL

Thomas L. Johnston, Bloomfield Hills, Raymond C. Boettner, Dearborn Heights, Richard H. Bush, Detroit, and Arthur J. McEvily, Jr., Dearborn, Mich., assignors to Ford Motor Company, Dearborn, Mich., a corporation of Delaware

Continuation-in-part of application Ser. No. 459,320, May 27, 1965. This application June 22, 1966, Ser. No. 560,049

6 Claims. (Cl. 148—12)

This application is a continuation-in-part of application Ser. No. 459,320 filed May 27, 1965, and assigned to the assignees of this application and now abandoned.

This invention is concerned with a high strength structural steel and the method by which this steel is produced. This high strength structural steel is weldable and in the as-rolled condition possesses a minimum yield strength of 80 K.s.i. and an impact energy absorption at  $-40^{\circ}$  F. of 40 foot pounds. This alloy is economical of expensive alloying ingredients and may be prepared either by air melting or vacuum melting techniques. No particular rolling procedures are required.

The unique properties of these high strength structural steels as compared to ordinary low alloy structural steel are readily apparent from a study of the three figures of drawing in which

FIGURE 1 is an electron beam transmission micrograph of the high strength structural steel of this invention. The structure is a massive martensite which is essentially ferrite containing a high density of dislocations. The magnification employed is  $\times 20,000$ . The chemistry of this sample is:

|                                 | Percent | 35 |
|---------------------------------|---------|----|
| Carbon                          | 0.02    |    |
| Nickel                          | 3.00    |    |
| Molybdenum                      | 3.00    |    |
| Manganese                       | 0.70    |    |
| Silicon                         | 0.30    | 40 |
| Niobium                         | 0.05    |    |
| Remainder essentially all iron. |         |    |

In this alloy both nickel and manganese serve to depress the austenite to massive martensite transformation temperature, while molybdenum serves to inhibit the transformation of austenite to equiaxed ferrite and pearlite prior to the transformation of austenite to massive martensite. The molybdenum may also serve as a carbide former. Chromium may be substituted in part for the more expensive molybdenum. To be commercially acceptable, each alloy should contain sufficient nickel or manganese or a combination of both metals to provide an acceptable austenite to massive martensite transformation temperature. The alloy should also contain a carbide forming metal which should be either chromium or molybdenum or a combination of these two metals which serves to inhibit the transformation of austenite to equiaxed ferrite and pearlite prior to the transformation temperature.

FIGURE 2 is a comparable electron beam transmission micrograph of a low alloy structural steel having a like thermal history. The structure is equiaxed ferrite containing a low density of dislocations. The magnification employed is  $\times 20,000$ . The nominal chemistry of this alloy is:

|                                 | Percent | 70 |
|---------------------------------|---------|----|
| Carbon                          | 0.02    |    |
| Nickel                          | 3.00    |    |
| Silicon                         | 0.30    |    |
| Manganese                       | 0.70    |    |
| Remainder essentially all iron. |         |    |

In contrast to heat treated alloy steels containing in excess of 0.1% carbon which derive their strength from quenched and tempered martensite or lower bainite, we have found that comparable yield strengths together with excellent impact toughness and weldability in the as-rolled condition can be obtained in very low carbon massive martensite steels. The carbon content of these steels should not exceed 0.07%. These steels are alloyed so as to transform on air cooling to massive martensite. The carbon content is minimized, and the alloying elements are selected to avoid the transformation to equiaxed ferrite during rolling or cooling. The austenite should be stable during processing. On subsequent cooling, the alloy should transform from austenite to massive martensite. The temperature at which this transformation takes place should not exceed  $1200^{\circ}$  F., and the preferred range is  $960$  to  $1150^{\circ}$  F. In general the yield strength varies inversely as the austenite to massive martensite transformation temperature.

The strength properties of air cooled plates are relatively insensitive to rolling temperatures below the austenite grain coarsening range at about  $1700$  to  $1800^{\circ}$  F. Impact properties are sensitive to the prior austenite grain size because the latter controls the density of grain boundary impurities. This dictates that excessive soaking times are to be avoided after completion of rolling at temperatures above  $1700^{\circ}$  F.

All heats were of one size, 20 lbs., with the exception of one 40 lb. heat, and were made in induction furnaces either in air or in vacuo. In air melts, chromium, manganese, silicon, molybdenum and carbon were added as ferro alloys. In vacuum melts, all alloying additions were in elemental form.

In air melts, after the melt down of the base charge of (Armco) iron, electrolytic nickel, and ferro-molybdenum, an addition of 0.05% aluminum was made. This addition was followed by ferro additions of chromium, manganese, silicon and vanadium, carbon and pure niobium as required. Prior to pouring at  $2800$ — $2850^{\circ}$  F., an additional 0.05% aluminum was added.

In vacuum melts, the starting charge was electrolytic iron and electrolytic nickel. After melt down in a vacuum of the order of 0.1 mm. Hg, an argon atmosphere at a pressure of 500 mm. Hg was introduced prior to the addition of manganese and silicon. Manganese has a high vapor pressure, and the presence of the argon atmosphere reduces its loss from the melt due to vaporization. The argon atmosphere was maintained while further additions of other desired elements were made and the melt poured.

For both air and vacuum melts, the ingots were cast in tapered chill molds with a mean diameter of  $2\frac{1}{8}$  inch and were allowed to cool in the molds at room temperature. After removal from the molds the ingots were sectioned transversely to provide two—ten pound cylinders for rolling. Both visual and X-ray examination of selected ingots indicated them to be essentially free of casting defects.

### ROLLING PROCEDURE

The usual rolling practice consisted of annealing the ingot halves at  $1775^{\circ}$  F. for 40 minutes after which they were box-rolled to 2 inch square bars using flat rolls with  $\frac{1}{8}$  inch reductions in roll opening and 5 minute reheat at  $1775^{\circ}$  F. after alternate passes. The bar temperature was not allowed to drop below  $1400^{\circ}$  in this stage. After box-rolling, the square bar was rolled to  $\frac{5}{8}$  inch plate either in the temperature range of  $1700$ — $1775^{\circ}$  F. with intermediate reheat, or was air cooled to  $1400^{\circ}$  F. and rolled without reheat. The finishing temperature in the latter case was approximately  $1350^{\circ}$  F. In both rolling sequences the resultant  $2 \times 14$  inch plate was air cooled to room temperature.

The mechanical properties such as yield strength, tensile strength, percent elongation and the reduction in area were determined on the basis of tensile tests of  $\frac{1}{8}$  inch diameter specimens. The elongation values were determined over a .8 inch gage length (7D), rather than over a usual 4D gage length. Hence the values obtained are about two-thirds that expected for a value measured over the smaller gage length.

The impact tests were made on standard 45°-V-notch

Charp bars. However, because of the large number of alloys investigated, complete transition curves were not always obtained. For purposes of screening, a single test at  $-40^{\circ}$  F. was often used.

5 Certain of the alloys which were produced in the investigation of this class of alloys are defined below in Table 1. In this table V indicates a vacuum melt and A an air melt.

TABLE 1

| Heat Number | Alloy Compositions, w/o |                |                |                  |                |                |                 |                |       |                   |                   |       | ° F. <sup>1</sup> |       |
|-------------|-------------------------|----------------|----------------|------------------|----------------|----------------|-----------------|----------------|-------|-------------------|-------------------|-------|-------------------|-------|
|             | C                       | Ni             | Mo             | Mn               | Cr             | Si             | Nb              | Al             | Ti    | V                 | P                 | S     | N                 | O     |
| VZ1736      | .0133                   | 2.98           | -----          | .68              | -----          | .32            | -----           | -----          | ----- | .001              | .007              | .003  | .001              | 1,304 |
| VZ1981      | <sup>2</sup> .01        | 3.05           | 2.54           | -----            | -----          | .39            | .062            | -----          | ----- | .001              | .006              | <.001 | .008              | 1,077 |
| VZ1996      | .0053                   | 3.05           | 2.85           | .73              | -----          | .46            | .060            | -----          | ----- | .002              | .005              | <.001 | .001              | 1,033 |
| VZ2009      | .0031                   | 3.08           | 1.85           | .73              | -----          | .43            | .055            | -----          | ----- | .001              | .005              | <.001 | .001              | ----- |
| VZ2010      | .0027                   | 3.05           | .95            | .75              | -----          | .41            | .050            | -----          | ----- | .003              | .008              | <.001 | .002              | 1,212 |
| VZ2011      | .004                    | 3.00           | 2.95           | .72              | -----          | .52            | -----           | .093           | ----- | .001              | .006              | <.001 | .003              | 1,156 |
| VZ2017      | .0193                   | 3.00           | 2.85           | .70              | -----          | .46            | .050            | -----          | ----- | .001              | .006              | <.001 | <.001             | 954   |
| VZ2038      | .0014                   | 3.30           | .63            | .72              | -----          | .30            | .040            | -----          | ----- | .001              | .008              | <.001 | .009              | 1,238 |
| AZ2039      | .0015                   | 2.90           | 2.70           | .50              | -----          | .23            | .030            | .035           | ----- | .012              | .013              | .005  | .010              | ----- |
| VZ2043      | .0019                   | 3.00           | 2.82           | .68              | -----          | .23            | .047            | -----          | ----- | .001              | .006              | <.001 | .006              | 1,041 |
| VZ2044      | .0386                   | 2.82           | 2.82           | .69              | -----          | .27            | .055            | -----          | ----- | .001              | .006              | <.001 | .002              | 958   |
| VZ2045      | <sup>2</sup> .02        | 3.12           | 1.40           | 1.52             | -----          | .29            | .045            | -----          | ----- | .001              | .006              | <.001 | .001              | 1,027 |
| VZ2052      | .0032                   | 2.95           | 2.75           | .65              | -----          | .30            | .030            | -----          | ----- | .001              | .008              | ----- | -----             | 1,060 |
| VZ2071      | .006                    | -----          | -----          | 2.40             | 2.90           | .27            | .065            | -----          | ----- | .003              | -----             | <.001 | -----             | ----- |
| VZ2072      | .049                    | -----          | 2.37           | 2.88             | .29            | .065           | -----           | -----          | ----- | .004              | -----             | <.001 | -----             | 1,197 |
| VZ2116      | .071                    | 2.93           | 2.79           | .69              | -----          | .28            | .049            | -----          | ----- | .001              | .007              | <.001 | .001              | ----- |
| VZ2117      | .0355                   | 2.96           | 1.98           | .72              | .95            | .34            | .046            | -----          | ----- | .002              | -----             | ----- | -----             | 957   |
| VZ2119      | <sup>2</sup> .02        | 2.90           | 2.75           | .65              | -----          | .39            | .075            | .11            | ----- | -----             | -----             | ----- | -----             | ----- |
| VZ2180      | <sup>2</sup> .03        | 2.85           | 2.70           | .67              | -----          | .22            | .080            | 20             | ----- | -----             | -----             | ----- | -----             | 1,112 |
| VZ2181      | .03                     | 2.95           | 2.82           | .67              | -----          | .39            | .080            | -----          | ----- | .49               | -----             | ----- | -----             | ----- |
| VZ2182      | .03                     | 2.85           | 2.80           | .67              | -----          | .39            | .075            | .10            | .50   | -----             | -----             | ----- | -----             | 1,065 |
| VZ2183      | .02                     | 2.85           | 2.75           | .67              | -----          | .41            | .070            | .10            | .18   | -----             | -----             | ----- | -----             | 1,082 |
| VZ2184      | .01                     | 2.90           | 2.75           | .67              | -----          | .38            | .080            | -----          | .18   | .50               | -----             | ----- | -----             | ----- |
| VZ2185      | <sup>2</sup> .02        | 2.95           | 2.70           | .67              | -----          | .38            | .075            | .070           | .18   | .49               | -----             | ----- | -----             | ----- |
| AZ2186      | .0108                   | 2.80           | 2.70           | .36              | -----          | .17            | .050            | .015           | ----- | .006              | .022              | ----- | -----             | ----- |
| AZ2187      | .0042                   | 2.80           | 2.70           | .53              | -----          | .24            | .070            | .080           | .11   | .005              | .022              | <.001 | -----             | 1,075 |
| AZ2188      | .0125                   | 2.85           | 2.65           | .48              | -----          | .22            | .065            | .075           | .19   | <sup>2</sup> .015 | <sup>2</sup> .015 | .0032 | -----             | ----- |
| AZ2189      | .0148                   | 2.80           | 2.75           | .58              | -----          | .25            | .065            | .075           | .14   | .005              | .020              | ----- | -----             | ----- |
| AZ2190      | .0104                   | 2.95           | 2.70           | .59              | -----          | .22            | .070            | .065           | ----- | .012              | .035              | .003  | .02               | 956   |
| AZ2191      | <sup>2</sup> .03        | 2.95           | 2.70           | .64              | -----          | .30            | .070            | .071           | .05   | .022              | .040              | .002  | .01               | ----- |
| AZ2192      | .0147                   | 2.95           | 2.70           | .64              | -----          | .24            | .060            | .070           | ----- | .022              | .041              | .002  | .02               | 1,006 |
| AZ2193      | <sup>2</sup> .03        | 2.95           | 2.65           | .59              | -----          | .22            | .050            | .080           | .12   | .26               | .023              | .040  | .002              | .01   |
| AZ2200      | .0261                   | 2.90           | 2.90           | .73              | -----          | .30            | .046            | -----          | ----- | .002              | -----             | <.001 | -----             | ----- |
| AZ2238      | .0138                   | 3.05           | 2.95           | .66              | -----          | .31            | .033            | -----          | ----- | .006              | -----             | .0023 | -----             | ----- |
| AZ2239      | .0170                   | 1.70           | 1.65           | 1.73             | 1.15           | .34            | .046            | .070           | ----- | .012              | -----             | .0033 | -----             | ----- |
| VZ2240      | .0497                   | 1.68           | 1.55           | 1.42             | 1.48           | .30            | .052            | -----          | ----- | .006              | -----             | .0015 | -----             | ----- |
| AZ2241      | .0127                   | 2.10           | 2.90           | .74              | -----          | .30            | .030            | .095           | ----- | .006              | -----             | .0032 | -----             | ----- |
| AZ2242      | .0142                   | 1.18           | 2.95           | .77              | -----          | .32            | .032            | .11            | ----- | .007              | -----             | .0032 | -----             | ----- |
| AZ2243      | .0423                   | 2.15           | 3.05           | .98              | .49            | .36            | .035            | .13            | ----- | .006              | -----             | .0034 | -----             | ----- |
| AZ2252      | .0177                   | -----          | -----          | 2.60             | 3.02           | .27            | .057            | .035           | ----- | .016              | -----             | <.001 | -----             | 903   |
| AZ2253      | .0194                   | -----          | -----          | 2.65             | 3.30           | .29            | .040            | .065           | ----- | .015              | -----             | .005  | .008              | 881   |
| AZ2260      | .0252                   | 3.10           | 2.10           | .81              | .99            | .35            | .045            | .15            | ----- | .012              | -----             | .003  | -----             | 916   |
| AZ2261      | .0369                   | 3.10           | 1.08           | .79              | .90            | .32            | .045            | .055           | ----- | .008              | -----             | .0022 | -----             | 951   |
| AZ2262      | .0301                   | 3.05           | 1.05           | .82              | 1.70           | .32            | .048            | .060           | ----- | .013              | -----             | .0022 | -----             | 914   |
| AZ2312      | <sup>2</sup> .09        | 1.95           | 1.10           | 1.88             | .49            | .29            | .020            | .020           | ----- | .011              | .017              | ----- | -----             | 935   |
| AZ2313      | .06                     | 4.00           | 1.00           | .96              | .46            | .32            | .02             | .020           | ----- | .011              | .018              | ----- | -----             | ----- |
| AZ2352      | <sup>2</sup> .05        | <sup>2</sup> 3 | <sup>2</sup> 3 | <sup>2</sup> 7   | -----          | <sup>2</sup> 3 | <sup>2</sup> 05 | <sup>2</sup> 1 | ----- | -----             | -----             | ----- | -----             | ----- |
| AZ2353      | <sup>2</sup> .05        | <sup>2</sup> 3 | <sup>2</sup> 3 | <sup>2</sup> 7   | -----          | <sup>2</sup> 3 | <sup>2</sup> 05 | <sup>2</sup> 1 | ----- | -----             | -----             | ----- | -----             | ----- |
| AZ2354      | <sup>2</sup> .05        | <sup>2</sup> 3 | <sup>2</sup> 3 | <sup>2</sup> 7   | -----          | <sup>2</sup> 3 | <sup>2</sup> 05 | <sup>2</sup> 1 | ----- | -----             | -----             | ----- | -----             | ----- |
| AZ2355      | <sup>2</sup> .05        | <sup>2</sup> 3 | <sup>2</sup> 3 | <sup>2</sup> 7   | -----          | <sup>2</sup> 3 | <sup>2</sup> 05 | <sup>2</sup> 1 | ----- | -----             | -----             | ----- | -----             | ----- |
| AZ2422      | .1040                   | -----          | -----          | 2.35             | 2.75           | .21            | .03             | .03            | ----- | .19               | .011              | .012  | .005              | .010  |
| AZ2423      | .0830                   | -----          | -----          | 2.28             | 2.90           | .14            | .03             | -----          | .18   | .011              | .014              | .014  | -----             | ----- |
| AZ2424      | .05                     | -----          | -----          | 2.56             | 3.00           | .27            | .05             | .04            | ----- | -----             | -----             | ----- | -----             | ----- |
| AZ2425      | .05                     | -----          | -----          | 2.56             | 3.02           | .27            | .05             | -----          | ----- | -----             | -----             | ----- | -----             | ----- |
| AZ2475      | .05                     | -----          | .52            | 2.30             | 2.33           | .08            | .040            | .040           | .040  | -----             | -----             | ----- | -----             | ----- |
| AZ2476      | .05                     | -----          | .55            | 2.58             | 3.00           | .14            | .055            | .048           | ----- | -----             | -----             | ----- | -----             | ----- |
| AZ2477      | .0134                   | -----          | -----          | 2.62             | 3.01           | .24            | .055            | .045           | ----- | .17               | .014              | .014  | .005              | .011  |
| AZ2519      | <sup>2</sup> .05        | -----          | -----          | 2.50             | 2.90           | .25            | .060            | -----          | ----- | .19               | -----             | ----- | -----             | ----- |
| AZ2520      | <sup>2</sup> .05        | -----          | -----          | 2.39             | 3.01           | .22            | -----           | -----          | ----- | .19               | -----             | ----- | -----             | ----- |
| AZ2553      | .0128                   | -----          | -----          | 2.62             | 3.05           | .32            | .055            | .040           | ----- | .19               | -----             | ----- | -----             | ----- |
| AZ2554      | .0163                   | -----          | -----          | 2.55             | 3.22           | .31            | .057            | -----          | ----- | .16               | -----             | ----- | -----             | ----- |
| AZ2555      | .0133                   | -----          | -----          | 2.54             | 3.20           | .28            | .060            | .035           | ----- | -----             | -----             | ----- | -----             | ----- |
| AZ2556      | .0154                   | -----          | -----          | 2.70             | 3.11           | .42            | -----           | -----          | ----- | .17               | -----             | ----- | -----             | ----- |
| AZ2557      | .0138                   | -----          | -----          | 2.60             | 3.03           | .34            | -----           | .035           | ----- | -----             | -----             | ----- | -----             | ----- |
| AZ2559      | <sup>2</sup> 0          | -----          | -----          | <sup>2</sup> 2.5 | <sup>2</sup> 3 | <sup>2</sup> 3 | -----           | <sup>2</sup> 1 | ----- | <sup>2</sup> 1    | -----             | ----- | -----             | ----- |

<sup>1</sup> Temperature at which Transformation Starts on Cooling. <sup>2</sup> Nominal composition.

Table 2 has been prepared to demonstrate the effect of rolling temperature upon certain of these alloys. 60

TABLE 2

| Heat Number | C, w/o | Si, w/o | Nb, w/o | Al, w/o | V, w/o | Rolling Temperature, ° F. | Y.S. (2%), K.S.I. | T.S. K.S.I. | ε, percent | R.A., percent | Charpy (-40° F.), ft.-lb. |
|-------------|--------|---------|---------|---------|--------|---------------------------|-------------------|-------------|------------|---------------|---------------------------|
| VZ2117      | -----  | -----   | -----   | -----   | -----  | 1,400                     | 108               | 139         | 12         | 71            | 222                       |
| VZ2191      | -----  | -----   | -----   | -----   | -----  | 1,750                     | 111               | 141         | 12         | 69            | 238                       |
| AZ2238      | -----  | -----   | -----   | -----   | -----  | 1,750                     | 113               | 137         | 12         | 57            | 26                        |
| AZ2239      | -----  | -----   | -----   | -----   | -----  | 1,400                     | 113               | 130         | 12         | 59            | 131                       |
| VZ2240      | -----  | -----   | -----   | -----   | -----  | 1,750                     | 110               | 131         | 11         | 69            | 126                       |
| AZ2243      | -----  | -----   | -----   | -----   | -----  | 1,750                     | 113               | 155         | 12         | 62            | 72                        |
| AZ2260      | -----  | -----   | -----   | -----   | -----  | 1,750                     | 115               | 153         | 12         | 63            | 140                       |
| -----       | -----  | -----   | -----   | -----   | -----  | 1,400                     | 115               | 142         | 11         | 45            | 178                       |
| -----       | -----  | -----   | -----   | -----   | -----  | 1,750                     | 114               | 148         | 11         | 54            | 100                       |
| -----       | -----  | -----   | -----   | -----   | -----  | 1,400                     | 115               | 144         | 11         | 57            | 44                        |
| -----       | -----  | -----   | -----   | -----   | -----  | 1,750                     | 111               | 142         | 11         | 67            | 36                        |
| -----       | -----  | -----   | -----   | -----   | -----  | 1,750                     | 111               | 142         | 11         | 67            | 61                        |

TABLE 2—Continued

| Heat Number         | C, w/o          | Si, w/o        | Nb, w/o | Al, w/o | V, w/o         | Rolling Temperature, °F. | Y.S., (2%), K s.i. | T.S., K s.i. | ε, percent | R.A., percent | Charpy (-40° F.), ft.-lb. |
|---------------------|-----------------|----------------|---------|---------|----------------|--------------------------|--------------------|--------------|------------|---------------|---------------------------|
| AZ2261              |                 |                |         |         |                | 1,400                    | 96                 | 127          | 12         | 59            | 59                        |
|                     |                 |                |         |         |                | 1,750                    | 99                 | 124          | 13         | 70            | 35                        |
| AZ2262              |                 |                |         |         |                | 1,400                    | 111                | 143          | 11         | 58            | 58                        |
|                     |                 |                |         |         |                | 1,750                    | 110                | 138          | 11         | 58            | 64                        |
| AZ2312              |                 |                |         |         |                | 1,400                    | 120                | 155          | 11         | 50            | 48                        |
|                     |                 |                |         |         |                | 1,750                    | 112                | 152          | 10         | 45            | 41                        |
| AZ2313              |                 |                |         |         |                | 1,400                    | 103                | 139          | 12         | 48            | 58                        |
|                     |                 |                |         |         |                | 1,750                    | 100                | 139          | 13         | 50            | 72                        |
| VZ2071              | .006            | .27            | .065    |         |                | 1,400                    | 67                 | 81           | 19         | 71            | 239                       |
| AZ2252              | .0177           | .27            | .057    | .035    |                | 1,400                    | 110                | 135          | 10         | 58            | 17                        |
| AZ2253              | .0194           | .29            | .040    | .065    |                | 1,400                    | 118                | 141          | 9          | 54            | 11                        |
|                     |                 |                |         |         |                | 1,700                    | 112                | 136          | 11         | 60            | 10                        |
| AZ2553              | .0128           | .32            | .055    | .040    | .19            | 1,400                    | 101                | 118          | 12         | 70            | 94                        |
| AZ2477              | .0134           | .24            | .055    | .045    | .17            | 1,400                    | 106                | 124          | 11         | 64            | 115                       |
| AZ2555              | .0135           | .28            | .060    | .035    |                | 1,400                    | 105                | 124          | 11         | 74            | 95                        |
| AZ2554              | .0163           | .31            | .057    |         | .16            | 1,400                    | 112                | 131          | 10         | 67            | 20                        |
| AZ2559              | <sup>1</sup> 0  | <sup>1</sup> 3 |         |         | <sup>1</sup> 1 | 1,400                    | 110                | 130          | 10         | 71            | 95                        |
| AZ2556              | .0154           | .42            |         |         | .17            | 1,400                    | 113                | 132          | 10         | 73            | 5                         |
| AZ2557              | .0138           | .34            |         |         | .085           | 1,400                    | 105                | 123          | 11         | 64            | 16                        |
| VZ2072              | .049            | .29            | .065    |         |                | 1,400                    | 102                | 128          | 11         | 72            | 11                        |
| AZ2425              | <sup>1</sup> 05 | .27            | .05     |         |                | 1,400                    | 117                | 149          | 12         | 67            | 135                       |
| AZ2424              | <sup>1</sup> 05 | .27            | .05     | .04     | .01            | 1,400                    | 114                | 143          | 11         | 72            | 150                       |
| AZ2422              | .1040           | .21            | .03     | .03     | .19            | 1,400                    | 143                | 176          | 10         | 54            | 13                        |
| AZ2423              | .0830           | .14            | .03     | .01     | .18            | 1,700                    | 136                | 171          | 11         | 59            | 14                        |
| AZ2519              | <sup>1</sup> 05 | .25            | .060    |         | .19            | 1,400                    | 140                | 176          | 10         | 53            | 21                        |
| AZ2520              | <sup>1</sup> 05 | .22            |         |         | .19            | 1,700                    | 132                | 170          | 11         | 49            | 8                         |
| AZ2475 <sup>2</sup> | <sup>1</sup> 05 | .08            | .040    | .040    | .13            | 1,400                    | 140                | 178          | 10         | 36            | 14                        |
| AZ2476 <sup>2</sup> | <sup>1</sup> 05 | .14            | .055    | .048    |                | 1,700                    | 135                | 171          | 11         | 50            | 18                        |
|                     |                 |                |         |         |                | 1,400                    | 141                | 167          | 11         | 55            | 17, 30, 14                |
|                     |                 |                |         |         |                | 1,700                    | 131                | 165          | 11         | 61            | 39, 21, 10                |
|                     |                 |                |         |         |                | 1,400                    | 143                | 180          | 10         | 60            | 17                        |
|                     |                 |                |         |         |                | 1,700                    | 134                | 173          | 10         | 61            | 25                        |
|                     |                 |                |         |         |                | 1,400                    | 133                | 175          | 11         | 62            | 22                        |
|                     |                 |                |         |         |                | 1,700                    | 132                | 172          | 11         | 65            | 13                        |
|                     |                 |                |         |         |                | 1,400                    | 130                | 169          | 10         | 64            | 36                        |
|                     |                 |                |         |         |                | 1,700                    | 128                | 167          | 11         | 64            | 30                        |
|                     |                 |                |         |         |                | 1,400                    | 141                | 179          | 11         | 64            | 27                        |
|                     |                 |                |         |         |                | 1,700                    | 139                | 179          | 11         | 64            | 30                        |

<sup>1</sup> Nominal composition. <sup>2</sup> 5 Mn addition.

Table 3 has been prepared to illustrate the effect of cooling at different rates from 1400° F.

microscopy is seen to consist of ferrite plates containing a high density of dislocations. Such a configuration of

TABLE 3  
[Alloy (VZ2052)—.0032C-2.95Ni-2.75Mo]

| Cooling Rate, °F. min. <sup>-1</sup> | Cooling Procedure                                            | Y.S., (2%), K s.i. | T.S., K s.i. | ε, Percent | R.A., Percent | Charpy (-40° F.), ft.-lb. |
|--------------------------------------|--------------------------------------------------------------|--------------------|--------------|------------|---------------|---------------------------|
| 1,400                                | Estimated for water quench following rolling.                | 100                | 109          | 12         | 77            | 238                       |
| 100                                  | Average for air cooling following rolling.                   | 99                 | 109          | 14         | 79            | 151                       |
| 6                                    | ½ hr. at 1775° F. followed by furnace cool at constant rate. | 94                 | 99           | 12         | 79            | 24                        |
| 2½                                   | Furnace cool following rolling.                              | 69                 | 89           | 24         | 78            | 239                       |

The results of tests of determine the effect of the rolling temperature on the mechanical properties are contained in Table 2. Below 1750° F. down to 1350° F., a range in which the alloys are austenitic, there appears to be little effect of the rolling temperature on the properties. For both the Mo-Ni alloy and the Cr-Mn alloy, yield strengths in excess of 100,000 p.s.i. are obtained. The impact values are higher in vacuum melts than in air melts, but in both cases the toughness is high as shown in FIGURE 3 where some of the present results are plotted and compared with the impact properties of T-1, 9Ni,<sup>(6)</sup> HY-80,<sup>(9)</sup> 5Ni-Cr-Mo-V,<sup>(9)</sup> and 1Mn<sup>(10)</sup> steels. The reduction in area of the low carbon alloys is high, a direct indication that particle effects in ductile fracture are small. In addition, a high reduction in area has often been correlated with a high value of the shelf energy.

The transformation product observed in both the 3Mo-3Ni and the 3Cr-2.5Mn alloys was predominantly massive martensite. The leaner alloys start to transform at higher temperatures and they contain a much greater proportion of equiaxed ferrite. Whenever equiaxed ferrite formed in large amounts, the transformation range was not only higher, but also much broader than that observed for a transformation to massive martensite. In FIGURE 1 the structure as examined by electron transmission

unpinned dislocations existing in a matrix relatively free of particles imparts both strength and toughness to the alloy. The macroscopic yield strength is strongly dependent upon the high strain hardening rate associated with such dislocation arrays. High toughness results from the ability of the dislocations to accommodate the imposed high strain rates of the Charpy test by rapid relaxation of stress concentrations. The relaxation rate depends in turn on the allowable plastic strain rate,  $\epsilon$ , which is a fraction of the density of dislocation,  $n$ , and their velocity  $v$ , as given by:

$$\epsilon = nbv \quad (9)$$

where  $b$  is the Burgers vector. A high initial value for  $n$  leads to a spreading out rather than a concentration of shear deformation, and reduces the average velocity of motion required. This latter effect is a particularly important consideration in iron based alloys at low temperatures where the velocity of motion of a dislocation as a function of stress decreases sharply. The influence of cooling rate on the mechanical properties is shown in Table 3 for 3Ni-3Mo steel. A rapid quench did not affect the tensile properties, but some improvement in toughness compared to air cooling was noted. If the alloy is very slowly cooled after rolling, the amount of equiaxed

ferrite will of course increase. The grain size is much larger than the needles of massive martensite. The appearance of the equiaxed structure is shown in FIGURE 2 for a 3Ni alloy. Examination of thin foils reveals a marked decrease in dislocation content as compared to massive martensite. As a consequence both the impact and tensile properties are lessened. Similarly, if the alloys are either reheated after rolling and held at a temperature high in the ferrite range (1200-1400° F.) or furnace cooled from the rolling temperature, there is a loss in strength. The properties as a function of tempering temperature are listed in Table 4.

TABLE 4.—EFFECT OF TEMPERING TEMPERATURE ON IMPACT TOUGHNESS

[Alloy (VZ1996)—0.053C-3.05Ni-2.85Mo Plate A rolled at 1250° F. and Plate B rolled with cooling from 1850° to 1700° F.]

| Condition | Temperature, °F. | Time, hr. | Hardness K.S.i. | Charpy ft.-lb. |
|-----------|------------------|-----------|-----------------|----------------|
| A         |                  |           | 61              | 240            |
| A         | 600              | 1         | 61              | 209            |
| A         | 1,000            | 1         | 62              | 240            |
| A         | 1,200            | 4         | 60              | 65             |
| A         | 1,400            | 1         | 50              | 240            |
| A         | 1,700            | 2         | 61              | 161            |
| A         | 1,900            | 1         | 60              | 9              |
| B         |                  |           | 62              | 69             |
| B         | 1,600            | 1         | 60              | 240            |
| B         | 1,700            | 1         | 61              | 86             |
| B         | 1,800            | 1         | 61              | 35             |

When the material is reaustenitized there is no loss in properties provided that the temperatures and times are such as to avoid grain coarsening. For example, the properties after heat treatment at 1700° F. are much superior to those obtained at 1900° F.

The effect of varying the carbon content on the mechanical properties of the base alloys, 3Ni-3Mo-.7Mn-3Si-.05Nb, and 2.5Mn-3Cr-3Si-.05Nb is shown in Table 5.

TABLE 5.—EFFECT OF CARBON CONTENT ON PROPERTIES

(A) Base Alloy 3Ni-3Mo Rolled at 1,400° F.

| Heat Number | C, w/o | Y.S., (2%), K.S.i. | T.S., K.S.i. | ε, Percent | R.A., Percent | Charpy ft.-lb., (-40° F.) |
|-------------|--------|--------------------|--------------|------------|---------------|---------------------------|
| VZ2043      | .0019  | 84                 | .96          | 15         | 71            | 170                       |
| VZ2052      | .0032  | 99                 | 109          | 14         | 79            | 151                       |
| VZ2229      | .0261  | 112                | 133          | 13         | 65            | 239                       |
| VZ2044      | .0386  | 108                | 135          | 12         | 71            | 175                       |
| VZ2017      | .0493  | 111                | 144          | 13         | 65            | 148                       |
| VZ2116      | .071   | 110                | 158          | 13         | 56            | 59                        |

(B) Base Alloy 3Cr-2.5Mn Rolled at 1,400° F.

|         | VZ2071 | .006 | 67  | 81 | 19 | 71  | 239 |
|---------|--------|------|-----|----|----|-----|-----|
| VZ2072  | .049   | 117  | 149 | 12 | 67 | 135 |     |
| AZ2253  | .0194  | 118  | 141 | 9  | 54 | 11  |     |
| AZ2555  | .0135  | 105  | 123 | 11 | 70 | 48  |     |
| AZ2477* | .0134  | 106  | 124 | 11 | 64 | 115 |     |

\*.1V addition.

These results show an increase in yield and tensile strengths with an increase in carbon content with air melted alloys generally stronger than those vacuum melted. The results of the impact tests are less straightforward. In vacuum melted 3Ni-3Mo alloys the impact strength remained high up to the 0.07 carbon level, but in the vacuum melted 2.5Mn-3Cr series there was a drop in impact resistance when the carbon level was increased even from .01 to .05. It is noteworthy that the addition of 0.1Al and 0.1V to air melt AZ2477 has increased the impact resistance at -40° F. to the 100 ft.-lb. range.

#### NICKEL AND MANGANESE

The results of a series of tests on 3Mo-.7Mn-3Si-.05Nb low carbon alloy heats in which the nickel content was varied are shown in Table 6.

TABLE 6.—EFFECT OF NICKEL CONTENT ON PROPERTIES  
[Base alloy—0.02C-3Mo rolled at 1400° F.]

| Heat Number | Ni, w/o | Y.S., (2%), K.S.i. | T.S., K.S.i. | ε, Percent | R.A., Percent | Charpy ft.-lb., (-40° F.) |
|-------------|---------|--------------------|--------------|------------|---------------|---------------------------|
| AZ2242      | 1.18    | 76                 | 88           | 16         | 60            | 14                        |
| AZ2241      | 2.10    | 87                 | 108          | 16         | 64            | 138                       |
| AZ2039      | 2.90    | 113                | 130          | 12         | 59            | 131                       |

It is seen that an increase of nickel content for the same carbon level leads to an increase in the strength properties. Except for heat AZ2242, all of these alloys possess an impact strength at -40° F. in excess of 100 ft.-lbs.

Results of a similar series of the 3Cr-Mn alloys in which the manganese content has been systematically varied have not been obtained. However, it is expected that the influence of manganese should be similar to that of nickel.

An important influence of molybdenum is to increase 20 hardenability, and since this can also be accomplished by an increase in the manganese content, several heats were made of a 3Ni alloy in which both the molybdenum and manganese contents were varied. The results are given in Table 7.

TABLE 7.—EFFECT OF MOYLBDENUM AND MANGANESE CONTENT ON PROPERTIES  
[Base alloy—0.02C-3Ni rolled at 1400° F.]

| Heat Number | Mo, w/o | Mn, w/o | Y.S., (2%), K.S.i. | T.S., K.S.i. | ε, Percent | R.A., Percent | Charpy ft.-lb., (-40° F.) |
|-------------|---------|---------|--------------------|--------------|------------|---------------|---------------------------|
| VZ1981      | 2.54    |         | 75                 | 87           | 17         | 83            | 238                       |
| VZ2045      | 1.40    | 1.52    | 91                 | 103          | 13         | 77            | 235                       |
| VZ2052      | 2.75    | .05     | 99                 | 109          | 14         | 79            | 151                       |

These results indicate that manganese alone (VZ1981) can lead to high toughness, but that in order for the 40 yield strengths to reach to 100K s.i. level, the presence of a carbide forming element (e.g., molybdenum) in this base alloy is needed.

#### MOLYBDENUM AND CHROMIUM

These two elements have a similar effect on properties. Both increase hardenability, but chromium is also effective in lowering the  $M_s$  temperature and both form alloy carbides in the same temperature range. These carbides are believed to form within the ferrite during the air cool after rolling.

The effect of molybdenum content on the properties is shown in Table 8.

TABLE 8.—EFFECT OF MOYLBDENUM CONTENT ON PROPERTIES  
[Base alloy—0.02C-3Ni rolled at 1400° F.]

| Heat Number | Mo, w/o | Y.S., (2%), K.S.i. | T.S., K.S.i. | ε, Percent | R.A., Percent | Charpy ft.-lb., (-40° F.) |
|-------------|---------|--------------------|--------------|------------|---------------|---------------------------|
| VZ1736*     |         | 47                 | 62           | 32         | -----         | 240                       |
| VZ2038      | .63     | 56                 | 70           | 23         | 75            | 113                       |
| VZ2010      | .05     | 68                 | 81           | 18         | 75            | 240                       |
| VZ2009      | 1.85    | 83                 | 93           | 16         | 72            | 240                       |
| VZ2052      | 2.75    | 99                 | 109          | 14         | 79            | 151                       |

\* $\frac{1}{8}$  inch rod heated at 1,650° F. for .5 hour and air cooled.

Over this range of molybdenum contents there is a monotonic increase in yield strength with increase in molybdenum content. The impact properties are a maximum in the 1-2% Mo range in this table; however, on occasion in alloys of higher molybdenum content with the same nominal compositions as VZ2052, e.g., VZ1996, impact values of 240 ft.-lbs. at -40° F. have been obtained.

The effects of chromium on the properties can be seen in the following Table 9.

TABLE 9.—EFFECT OF CHROMIUM CONTENT ON PROPERTIES

[Base alloy—0.05C-1.5Ni-1.5Mo-1.5Mn rolled at 1,400° F.]

| Heat Number | Cr, w/o | Y.S., (2%), K s.i. | T.S., K s.i. | $\epsilon$ , Percent | R.A., Percent | Charpy, ft.-lb. |
|-------------|---------|--------------------|--------------|----------------------|---------------|-----------------|
| VZ2240      | 1.48    | 113                | 155          | 12                   | 63            | 140             |
| AZ2239      | 1.15    | 110                | 134          | 11                   | 59            | 58              |
| AZ2312      | .5      | 120                | 155          | 10                   | 50            | 48              |

TITANIUM—ALUMINUM—VANADIUM—  
NIOBIUM

The effects of small additions of elements such as Ti, Al, V and Nb are difficult to specifically isolate because

5 concerned. Any loss in hardenability due to the refinement of austenitic grain size does not appear to be significant in these alloys. In the vacuum melts there is no beneficial effect imparted by the addition of elements Ti, V and Al. In fact these additions can reduce the yield strength (e.g., VZ2185). This reduction may be due to the complete removal from solution of carbon by vanadium. In air melts, the addition of vanadium to alloys low in phosphorus and sulfur, has a beneficial effect on yield strength and the impact properties at -40° F. remain high (AZ2188). In fact the properties of all of the air melts are good, with the exception of AZ2192 which showed a reduction in impact strength for a high phosphorus and vanadium content. The addition of Ti and Al to air melts appears to be beneficial. Results of a similar study with Cr-Mn alloys are shown in Table 11.

TABLE 11.—EFFECT OF VANADIUM, ALUMINUM AND NIOBIUM CONTENT ON PROPERTIES

[Base alloy—0.05C-3Cr, 2.5Mn rolled at 1,400° and 1,750° F.]

| Heat Number | V, w/o | Al, w/o | Nb, w/o | Rolling Temperature, °F. | Y.S., (2%), K s.i. | T.S., K s.i. | $\epsilon$ , Percent | R.A., Percent | Charpy, (-40° F.), ft.-lb. |
|-------------|--------|---------|---------|--------------------------|--------------------|--------------|----------------------|---------------|----------------------------|
| AZ2477      | .17    | .045    | .05     | { 1,400<br>1,750         | 106<br>105         | 124<br>124   | 11<br>11             | 64<br>74      | 115<br>95                  |
| AZ2553      | .19    | .040    | .055    | { 1,400<br>1,750         | 101<br>99          | 117<br>115   | 12<br>11             | 70<br>74      | 94<br>116                  |
| AZ2554      | .16    | —       | .057    | { 1,400<br>1,750         | 112<br>110         | 131<br>130   | 10<br>10             | 67<br>71      | 20<br>95                   |
| AZ2555      | —      | .035    | .060    | { 1,400<br>1,750         | 105<br>100         | 123<br>117   | 11<br>11             | 70<br>76      | 48<br>100                  |
| AZ2556      | .17    | —       | —       | { 1,400<br>1,750         | 118<br>113         | 142<br>135   | 10<br>10             | 64<br>72      | 16<br>11                   |
| AZ2557      | —      | .035    | —       | { 1,400<br>1,750         | 107<br>102         | 128<br>121   | 11<br>11             | 73<br>75      | 41<br>15                   |

of the many complex interactions possible. These elements have been generally added in quantities consistent with usual alloy steel practice. Throughout this investigation Nb has been a standard alloying element in the amount of 0.05 w/o. This usage of Nb is based upon preliminary work with rod material which revealed both an increase in the yield strength as well as the impact strength of alloys containing .02 w/o C. This effect of Nb can also be seen in the data for alloys VZ2011 and VZ2180, Table 10.

40 The properties of the first two heats indicate that the attainment of high impact strengths in Cr-Mn alloys is reproducible. These properties compare favorably with those of 3Mo-3Ni air melts. The omission of either vanadium or aluminum does not adversely affect the properties provided that the rolling temperature is at least 1700° F. (Heats AZ2555 and AZ2554.) The higher rolling temperature may facilitate the removal from solution 45 of nitrogen by these elements. The absence of Nb leads to

TABLE 10.—EFFECT OF TITANIUM, ALUMINUM, VANADIUM AND NIOBIUM CONTENT ON PROPERTIES

[Base alloy—3Ni-3Mo rolled at 1,400° F.]

| Heat Number | C, w/o | Ti, w/o | Al, w/o | V, w/o | Nb, w/o | Y.S., (2%), K s.i. | T.S., K s.i. | $\epsilon$ , percent | R.A., percent | Charpy, (-40° F.), ft.-lb. |
|-------------|--------|---------|---------|--------|---------|--------------------|--------------|----------------------|---------------|----------------------------|
| VZ2011      | .004   | .093    | —       | —      | .080    | 83                 | 96           | 17                   | 72            | 238                        |
| VZ2180      | *.03   | .20     | —       | —      | .080    | 98                 | 108          | 15                   | 73            | 238                        |
| VZ2181      | *.03   | —       | —       | .49    | .080    | 95                 | 107          | 16                   | 74            | 239                        |
| VZ2182      | *.03   | —       | .10     | .50    | .075    | 88                 | 100          | 19                   | 71            | 239                        |
| VZ2183      | *.02   | .18     | .10     | —      | .070    | 88                 | 101          | 17                   | 74            | 238                        |
| VZ2184      | *.01   | .18     | —       | .50    | .080    | 81                 | 94           | 19                   | 67            | 239                        |
| VZ2185      | *.02   | .18     | .070    | .49    | .075    | 83                 | 95           | 18                   | 68            | 207                        |
| VZ2229      | .0261  | —       | —       | —      | .046    | 112                | 133          | 13                   | 65            | 239                        |
| AZ2187      | .0042  | .11     | .080    | —      | .070    | 102                | 115          | 13                   | 67            | 117                        |
| AZ2188      | .0125  | —       | .075    | .19    | .065    | 116                | 128          | 12                   | 65            | 122                        |
| AZ2191      | *.03   | .05     | .071    | —      | .070    | 116                | 139          | 11                   | 56            | 91                         |
| AZ2192      | .0147  | —       | .070    | .23    | .060    | 122                | 135          | 11                   | 61            | 34                         |
| AZ2193      | *.03   | .12     | .080    | .26    | .050    | 111                | 125          | 13                   | 57            | 186                        |
| AZ2039      | .0015  | —       | .085    | —      | .080    | 110                | 127          | 11                   | 58            | 126                        |

\*Nominal.

The addition of Nb raises the yield strength and does not impair impact properties at -40° F. This effect of Nb is thought to be due to its role in refining the grain size of austenite. In these low carbon alloys not enough of the NbC phase is formed to adversely affect impact strength as has been found in the case of higher carbon alloys. Refinement of the grain size of the austenite will result in a smaller needle length of the massive martensite, and will also tend to distribute impurity particles over a larger total grain boundary surface area. Both of these effects will be beneficial insofar as toughness is

65 a decrease in impact resistance, particularly at the higher rolling temperature (Heats AZ2556 and AZ2557).

THE EFFECT OF PHOSPHORUS AND SULFUR

70 The amount of phosphorus and sulfur in these alloys was generally kept to less than 0.015 percent each. In order to determine the effects of these elements in larger quantities, a series of air melted alloys was prepared with phosphorus contents of up to .022 percent and sulfur up to 0.040 percent. The properties of these alloys are listed in Table 12.

TABLE 12.—EFFECT OF PHOSPHORUS AND SULFUR CONTENT ON PROPERTIES  
[Base alloy—0.02C-3Ni-3Mo rolled at 1,400° F.]

| Heat Number | P, w/o | S, w/o | Ti, w/o | Al, w/o | V, w/o | Nb, w/o | Y.S.,<br>(.2%),<br>K s.i. | T.S.,<br>K s.i. | $\epsilon$ ,<br>Percent | R.A.,<br>Percent | Charpy<br>(-40° F.),<br>ft.-lb. |
|-------------|--------|--------|---------|---------|--------|---------|---------------------------|-----------------|-------------------------|------------------|---------------------------------|
| AZ2039      | .012   | .013   | —       | .035    | —      | .030    | 110                       | 127             | 11                      | 58               | 126                             |
| AZ2190      | .012   | .035   | —       | .065    | —      | .070    | 117                       | 127             | 11                      | 56               | 126                             |
| AZ2187      | .005   | .022   | .11     | .080    | —      | .070    | 102                       | 115             | 13                      | 67               | 117                             |
| AZ2191      | .022   | .040   | .05     | .076    | —      | .070    | 116                       | 139             | 11                      | 56               | 91                              |
| AZ2188      | *.015  | *.015  | —       | .075    | .19    | .065    | 116                       | 128             | 12                      | 65               | 122                             |
| AZ2192      | .022   | .041   | —       | .070    | .23    | .060    | 122                       | 135             | 11                      | 61               | 34                              |
| AZ2189      | .005   | .020   | .14     | .075    | .41    | .065    | 89                        | 101             | 16                      | 67               | 118                             |
| AZ2193      | .023   | .040   | .12     | .080    | .26    | .050    | 111                       | 125             | 13                      | 57               | 186                             |

\*Estimated.

The effect of these additions is not systematic, but it is seen that these elements can reduce the CVN values. Titanium appears to have an effect which offsets the detrimental influence of phosphorus and sulfur on toughness.

## HARDENABILITY

In order to obtain an indication of the hardenability of these alloys a 2½ inch diameter ingot (AZ2531B) was sectioned in the transverse direction after casting. A hardness traverse across the diameter of the exposed face was made and the hardness values were found to vary in a random manner from 18½ to 19½ Rc. A similar traverse was made on a section through the ingot which had been reaustenitized and air cooled from 1750° F. and similar readings were obtained. The alloy is therefore fully hardened in section sizes at least up to 2½ inch diameter in both the as-cast and the air cooled conditions.

## WELDABILITY

The purposes of some initial tests on weldability were to determine if sound welds, free of cracks and blow holes could be obtained by standard welding techniques, and to assess the behavior of the heat affected zone. The welding was performed by members of the Manufacturing Development Staff. Test weldments were made using .02C-3Ni-3Mo steel plates.

The weld material was either of the same compositions as the plate with which a 75% argon-25%  $\text{CO}_2$  atmosphere was used, or Airco No. 352, low hydrogen, covered electrodes. The results of tests listed in Table 13 indicated that crack free welds can be obtained and that the heat affected zone is still quite tough, absorbing 44 to 104 ft.-lbs. Studies with 5Ni steels indicate that the transformation temperature of the present steels is sufficiently high to avoid cracking of the weld metal interface on cooling. Furthermore, the low carbon level prevents the formation of carbides which are known to have an embrittling effect.

15 the high reduction of area of the low carbon massive martensitic steels is indicative of good formability.

## EFFECT OF COLD WORK

A plate of 3Ni-3Mo-.02C alloy was reduced 84% by rolling at room temperature. The yield strength of the alloy was 240K s.i., its tensile strength was 207K s.i. and the elongation in 2" was 3%, as determined on flat tensile strips. The material still appeared tough in the sense that failure was not brittle; and occurred as a result of plastic instability with considerable lateral contraction in the immediate vicinity of the fracture.

## INGOT SIZE AND TRANSVERSE PROPERTIES

One 40 lb. heat of a 3Mo-3Ni-.02C alloy was vacuum melted and rolled to 5/8" plate thickness in order to make 30 a comparison with the properties of the usual 20 lb. heats. The width of the plate was 4 inches which permitted transverse as well as longitudinal properties to be obtained. The results were as follows:

|                 | Y.S.,<br>K s.i. | TS,<br>K s.i. | Percent<br>$\epsilon$ | Percent<br>R.A. |
|-----------------|-----------------|---------------|-----------------------|-----------------|
| Longitudinal    | 88              | 99            | 15                    | 79              |
| Long transverse | 95              | 106           | 14                    | 81              |

## IMPACT PROPERTIES

|                                                        | Orientation of Notch | Test Temperature |       |
|--------------------------------------------------------|----------------------|------------------|-------|
|                                                        |                      | -40°             | -120° |
| Transverse and parallel to rolling plane,<br>ft.-lb.   | —                    | 236              | 186   |
| Perpendicular to rolling plane, ft.-lb.                | —                    | 186              | 144   |
| Longitudinal and parallel to rolling plane,<br>ft.-lb. | —                    | 153              | 127   |

These results indicate about the usual sort of anisotropy associated with rolled plate products. The lower than usual value of 88K s.i. for the yield strength of the alloy 50 is thought to be due more to variation in carbon content than to a loss in tensile properties as a result of increasing the size of the ingot from 20 to 40 lbs.

TABLE 13.—EFFECT OF WELDING ON IMPACT TOUGHNESS  
[Base alloy—0.02C-3Ni-3Mo rolled at 1,400° F.]

| Charpy Notch Position Relative to Weld        | VZ2179-9<br>base <sup>1</sup> | VZ2179-4<br>352 | AZ2186-7<br>base <sup>1</sup> | AZ2186-8<br>Base <sup>1</sup> | AZ2186-6<br>352 | AZ2188-2<br>Base <sup>1</sup> | AZ2188-5<br>352 |
|-----------------------------------------------|-------------------------------|-----------------|-------------------------------|-------------------------------|-----------------|-------------------------------|-----------------|
| 1. Notch in weld adjacent parent metal        | 250                           | 89              | 72                            | 26                            | 47              | 217                           | 48              |
| 2. Same as 1                                  | 29                            | 100             | 29                            | 22                            | 104             | 221                           | 44              |
| 3. Notch in parent metal removed from<br>weld | 240                           | 240             | 141                           | 25                            | 139             | 80                            | 112             |
| 4. Notch in center of weld                    | 212                           | 6               | 16                            | 28                            | 14              | 12                            | 8               |

<sup>1</sup> Holes and cracks present in weldment.<sup>2</sup> Partial fracture along weld interface.

## FORMABILITY

In order to determine the formability of these alloys, 70 a ½ inch plate of the 3Ni-3Mo alloy was bent about a ½ inch diameter through an angle of 90°. No cracking was observed. A correlation between the formability of high strength alloys and the reduction of area in the tensile test has been established, and on this basis also 75

## AS CAST PROPERTIES

In many potential applications of high strength steels it may be desired to obtain the strength and toughness in the as-cast condition. In order to determine as-cast properties therefore, the following alloys, containing additions of either Zr or Hf for deoxidation, were cast and mechanical properties determined, Table 14.

TABLE 14.—EFFECT OF HAFNIUM AND ZIRCONIUM CONTENT ON AS-CAST MATERIAL  
[Base alloy—.05C-3Ni-3Mo]

| Heat Number | Hf,* w/o | Zr,* w/o | Y.S. (.05%),<br>K s.i. | T.S., K s.i. | $\epsilon$ , percent | R.A., percent | Charpy (-40° F.), ft.-lb. |
|-------------|----------|----------|------------------------|--------------|----------------------|---------------|---------------------------|
| AZ2352      | .05      | -----    | 109                    | 130          | 5                    | 10            | 16                        |
| AZ2353      | -----    | .05      | 110                    | 137          | 7                    | 14            | 9                         |
| AZ2354      | .01      | -----    | 110                    | 132          | 7                    | 14            | 14                        |
| AZ2355      | -----    | .01      | 90                     | 135          | 5                    | 12            | 13                        |

\*Nominal composition.

The strengths of these as-cast alloys are similar to the alloys as-rolled, but there is a sharp decline in impact and ductility values. Nevertheless the properties seem to be of sufficient interest to warrant further investigation.

The effect of a normalizing treatment on several other cast alloys was also studied, Table 15.

(3) Johnston, T. L., Stoloff, N. S., and Davies, K. G., Phil Mag., 12, 1965, p. 305.

(4) Manganello, S. J., Dabkowski, D. S., Porter, L. F., and Gross, J. H., Metals Engineering Quarterly, 5, No. 1, Feb. 1965, p. 1.

TABLE 15.—EFFECT OF NORMALIZING TREATMENT ON PROPERTIES OF AS CAST MATERIAL  
[Base alloy—.02C-3Ni-3Mo held  $\frac{3}{4}$  hr. at temperature]

| Normalizing Temperature<br>Heat Number | As Cast                            |                              | 1,800° F.                          |                              | 1,900° F.                          |                              | 2,100° F.                          |                              |
|----------------------------------------|------------------------------------|------------------------------|------------------------------------|------------------------------|------------------------------------|------------------------------|------------------------------------|------------------------------|
|                                        | Hardness, Rc<br>(-40° F.), ft.-lb. | Charpy<br>(-40° F.), ft.-lb. | Hardness, Rc<br>(-40° F.), ft.-lb. | Charpy<br>(-40° F.), ft.-lb. | Hardness, Rc<br>(-40° F.), ft.-lb. | Charpy<br>(-40° F.), ft.-lb. | Hardness, Rc<br>(-40° F.), ft.-lb. | Charpy<br>(-40° F.), ft.-lb. |
| VZ2180                                 | 17                                 | 5                            | 16                                 | 4                            | 17                                 | 5                            | 17                                 | 6                            |
| VZ2181                                 | 17                                 | 6                            | 14                                 | 6                            | 17                                 | 5                            | 18                                 | 5                            |
| AZ2190                                 | 22                                 | 8                            | 20                                 | 9                            | 21                                 | 8                            | 22                                 | 8                            |
| AZ2192                                 | 25                                 | 6                            | 22                                 | 5                            | 23                                 | 7                            | 21                                 | 9                            |

These results reveal that normalizing above 1800° F. has no significant effect upon the properties. The effect of lower normalizing temperatures is being investigated.

#### FATIGUE PROPERTIES

Fatigue tests were performed on a 3Ni-3Mo alloy having a yield strength and tensile strength of 112K s.i. and 133K s.i., respectively. Both smooth and notched specimens were tested as rotating beams (R. R. Moore type). The unnotched fatigue strength obeys the usual rule in that the fatigue endurance at long lives is about  $\frac{1}{2}$  of the tensile strength. The notched specimen (theoretical notch factor of 5) exhibits about the same degree of reduction of fatigue strength as other steels of this strength level.

Because of the uniform structure of this steel it is expected that the degree of scatter of fatigue data should be less than usual at these strength levels.

Preliminary fatigue crack growth studies in sheet specimens revealed a characteristic of these steels associated with the high impact toughness. The cracks grew until the stress on the remaining section was equal to the tensile strength of unnotched material, so that the material, statically, was notch insensitive.

#### CARBURIZATION

In certain instances it may be desired to increase the surface hardness by carburization. The effect on the properties of a carburized .02C-3Ni-3Mo alloy (Z1755) was therefore investigated. The carburization was done by the packed method at 1700° F. for 2 hrs. The resultant surface hardness was 55 Rc and that of the interior was 20 Rc. In one case the notch was present prior to carburizing and this specimen absorbed 17 ft.-lbs. in the Charpy impact test. In a second set of specimens, the notch was machined after carburization so that the base of the notch was in a noncarburized region. These specimens absorbed 95-155 ft.-lbs., indicating that the core of the specimen retains its toughness after this heat treatment.

The following partial bibliography is presented to assist in the understanding of this invention and its technical background.

#### REFERENCES

- (1) Rinebolt, J. A., and Harris, W. J., Jr., Trans. ASM, 44, 1952, 225.
- (2) McMahon, C. J., and Cohen, M., Acta Met., 13, 1965, 591.

(5) Marschall, C. W., Hehemann, R. F., and Troiano, A. R., Trans. ASM, 55, 1962, p. 135.

(6) McEvily, A. J., and Bush, R. H., unpublished results.

(7) McEvily, A. J., Ku, R. C., and Johnston, T. L., Trans. AIME, 236, 1966, p. 108.

(8) Owen, W. S., Wilson, E. A., Bell, T., in High Strength Materials, ed by V. Zackay, John Wiley and Sons, New York, 1965, p. 167.

(9) Rolfe, S. T., Haak, R. P., and Gross, J. H., Metals Engineering Quarterly, 5, No. 1, Feb. 1965, p. 33.

(10) Kube, L. J., Metals Progress, 88, 1965, p. 78.

(11) Davies, R. G., unpublished results.

(12) International Nickel Co. pamphlet, ZOM 4-65-4342, 1965.

(13) Kaufman, L., and Ringwood, A. E., Acta Met. 9, 1961, p. 941.

(14) Morrison, W. B., J. Iron and Steel Inst., 201, 1963, p. 317.

(15) Steel, 150, No. 2, Jan. 10, 1966, p. 67.

(16) Metals Progress, 88, No. 2, August 1965.

(17) Cottrell, A. H., Dislocations and Plastic Flow in Crystals, Oxford, 1953.

(18) Petch, N. J., Phil Mag., 1, 1956, p. 186.

(19) Meakin, J. D., and Petch, N. J., Symposium on Role of Substructure, 1963, ASD-TDR-63-324, p. 243.

(20) Ku, R. C., McEvily, A. J., and Johnston, T. L., to be published.

Being not unmindful of the following patents, 2,707,680, Succop, May 3, 1955; 3,044,872, Hayes, July 17, 1962; 3,135,600, Hardwick et al., June 2, 1964; and 703,911 (British), Feb. 10, 1954, we claim as our invention:

1. The process of producing a weldable structural steel object having in the as-rolled condition, a massive martensitic structure essentially free of equiaxed ferrite, a minimum yield strength of 80K s.i. and a minimum impact energy absorption value at -40° F. of 40 foot pounds comprising fabricating an alloy having a maximum carbon content of 0.07%, a content of alloying metal selected from the group consisting of nickel, molybdenum, chromium, manganese and silicon in an amount not substantially in excess of 7%, the sum of combinations of the nickel, molybdenum, chromium and manganese not exceeding about 6%, the alloy containing significant amounts of metal selected from the group consisting of nickel, manganese and combinations of nickel and manganese such that the transformation of austenite to massive martensite is retarded at temperatures above 1300°

F., the alloy further containing significant amounts of metal selected from the group consisting of chromium, molybdenum and combinations of chromium and molybdenum such that the transformation of austenite to equiaxed ferrite is essentially absent at temperatures above the austenite to massive martensite transformation temperature, the chemistry of the object being adjusted to exhibit an austenite to massive martensite transformation temperature below 1300° F. and a rate of transformation of austenite to massive martensite such that essentially no equiaxed ferrite is produced in air cooling from the austenite to massive martensite transformation temperature to room temperature, hot working the alloy and finishing the hot working operation at a temperature sufficiently low to inhibit substantial austenite grain growth during working and cooling down to the austenite to massive martensite transformation temperature, said object exhibiting a microstructure of massive martensite containing a high density of dislocations and metallurgically indistinguishable from the structure in FIGURE 1.

2. The process recited in claim 1 in which the alloy contains about 0.05% niobium.

3. A weldable structural steel object having in the as-rolled condition a massive martensitic structure essentially free of equiaxed ferrite, a minimum yield strength of 80K s.i. and a minimum impact energy absorption value at -40° F. of 40 foot pounds, a maximum carbon content of 0.07%, a content of alloying metal selected from the group consisting of nickel, molybdenum, chromium, manganese and silicon in an amount not substantially in excess of 7%, the sum of combinations of the nickel, molybdenum, chromium and manganese not exceeding about 6%, the alloy containing significant amounts of metal selected from the group consisting of nickel, manganese and combinations of nickel and manganese such that the transformation of austenite to massive martensite is retarded at temperatures above 1300° F., the alloy fur-

ther containing significant amounts of metal selected from the group consisting of chromium, molybdenum and combinations of chromium and molybdenum such that the transformation of austenite to equiaxed ferrite is essentially absent at temperatures above the austenite to massive martensite transformation temperature, the chemistry of the object being adjusted to exhibit an austenite to massive martensite transformation temperature below 1300° F. and a rate of transformation of austenite to massive martensite such that essentially no equiaxed ferrite is produced in air cooling from the austenite to massive martensite transformation temperature to room temperature, and exhibiting a microstructure of massive martensite containing a high density of dislocations and being metallurgically indistinguishable from the structure shown in FIGURE 1.

4. The weldable structural steel object recited in claim 3 and which includes a niobium content of about 0.05%.

5. The process recited in claim 1 in which the chromium, manganese, nickel and molybdenum are present in approximately equal amounts.

6. The object recited in claim 3 in which the chromium, manganese, nickel and molybdenum are present in approximately the same amounts.

#### References Cited

#### UNITED STATES PATENTS

3,132,025 5/1965 Hurley ----- 148-36 X

#### FOREIGN PATENTS

703,911 2/1954 Great Britain.

HYLAND BIZOT, *Primary Examiner.*

DAVID L. RECK, *Examiner.*

H. SAITO, W. W. STALLARD, *Assistant Examiners.*